

W. R. BOSSINGER.

INGOT MOLD.

APPLICATION FILED FEB. 14, 1913.

1,070,106.

Patented Aug. 12, 1913.



Witnesses:

Harry E. Davis  
Ben Anthony

Fig. 4. Inventor:

William. R. Bossinger

# UNITED STATES PATENT OFFICE.

WILLIAM R. BOSSINGER, OF MARION, OHIO.

## INGOT-MOLD.

1,070,106.

Specification of Letters Patent. Patented Aug. 12, 1913.

Application filed February 14, 1913. Serial No. 748,471.

*To all whom it may concern:*

Be it known that I, WILLIAM R. BOSSINGER, a citizen of the United States, residing in Marion, in the county of Marion and State of Ohio, have invented or discovered certain new and useful Improvements in Ingot-Molds, of which the following is a specification.

My invention relates particularly to that type of molds, wherein are cast iron or steel ingots or other castings.

The primary object of my invention is to provide a mold that will produce solid ingot castings which will be practically free from all blow-holes, pipes, cavities, segregation and other defects usually found in such castings.

A further object of my invention is to provide a mold that will be artificially cooled in one portion, will possess normal radiation in another portion, and in the remaining portion will be so designed as to artificially retard radiation and to permit the chemical creation of heat therein.

Other objects and advantages of the invention will be apparent during the course of the following description.

In the accompanying drawings, forming a part of this specification and in which like letters are employed to designate like parts throughout the same, Figure 1 shows a vertical section of my mold with an ordinary base. Fig. 2 shows a transverse section of my mold at the line Y—Y in Fig. 1, looking from above. Fig. 3 is a view of the top of the mold. Fig. 4 shows a vertical section of that part of the mold from the line Y—Y in Fig. 1, downward, but of a somewhat different design. In this modified form, the cooling cavities are horizontal instead of vertical as in Fig. 1, and Fig. 5 shows a transverse sectional view of the quadrangular passage F.

For purposes of explanation, my mold is divided into three portions or zones, each portion or zone being differentiated from the other two, by a different construction of its walls.

In the drawings, wherein is illustrated a preferred embodiment of my invention, the lower portion of the mold is represented by the zone A, which zone includes that portion of the mold from the line Y—Y in Fig. 1 to the bottom thereof. In this zone, the mold has a base D, an inlet E, a quadrangu-

lar passage F, inner side-walls G, outer side-walls I, spaces or cavities between said side-walls, designated by the letter H, and exhausts J. The side-walls G have inner surfaces K, and outer surfaces K<sup>1</sup>. The side-walls I have outer surfaces L and inner surfaces L<sup>1</sup>, all as shown in Fig. 1. The outer surfaces K<sup>1</sup> of the side-walls G, and the inner surfaces L<sup>1</sup> of the side-walls I, merge together at the mold bottom Z, at the corners N and at the zone top Y, forming thereby the inclosing walls of the said cavities H, substantially as shown in Figs. 1 and 2. The inlet E communicates directly with the continuous passage F, which, in turn, communicates directly with the various cavities H. Each of the four sides of the mold may have a single cavity H, or two or more smaller cavities separated from each other by partitions H<sup>1</sup>, which last preferred design is shown in Fig. 2. Each cavity may have its own exhaust J, or as in the preferred design shown in the drawings, the partitions H<sup>1</sup> are not extended fully to the zone top Y, thereby causing all of the cavities H in any one side of the mold to open into one general cavity communicating directly with the exhaust J. The said cavities H may also extend entirely around the inner wall G and be a simple upward extension of the passage F.

In a mold constructed as above mentioned, cold water, air or other cooling compound may be forced through the inlet E into the passage F, and by the constant renewal of such cooling compound compelled to continue upward into the cavities H and out through the exhausts J. The said walls G and I will be thus in uninterrupted contact with the cooling compound in the cavities H and thereby cause the temperature of said walls to be subjected to gradual reduction, effecting thereby a greater radiation of heat from that portion of the casting included in this zone.

The middle portion of my mold is represented by the zone B and includes that portion of the mold from the line Y—Y to the line X—X, as shown in Fig. 1. In this zone, the mold has side walls M with interior surfaces K and outer surfaces L. Said walls are normal and the heat radiation through same slower than in the zone A. In use, such slower radiation causes that portion of the casting contained in the

said zone B to remain in a molten state longer than the portion contained in the zone A, with the result that the force of gravity will cause the still molten metal, in the zone B to flow into all cavities, pipes, and the like existing in the portion of the casting contained in the zone A, and thereby eliminate these defects.

The upper portion of my mold is represented by the zone C, and includes all that part of the mold above the line X—X, as shown in Fig. 1. In this zone, the mold has main side-walls P, a refractory lining R, handles O and cover fasteners S. The side-walls P are of the same material and construction as the walls in the zone B, but have recesses cut in the interior surfaces thereof to receive the lining R which may consist of fire-brick, clay or other refractory substance, all as shown in Fig. 1. This refractory lining will retain the heat, and cause the metal of the casting to remain in a fluid or molten state longer than it otherwise would, with the result, that as explained above with reference to the zone B, the force of gravity will cause the still molten metal in the said zone C to flow into all cavities, pipes etc. existing in the cooler portion of the casting in the zone B, and thereby eliminate these defects.

The handles O are metal protuberances to which may be attached the ordinary forms of stripping machinery.

The interior of the mold is of a modified conical form, so that the diameter of the casting will be greater at the bottom than at the top, enabling the mold to be stripped from the casting without inversion.

Fig. 4 represents a different design of the zone A, in which the cavities or passages which convey the cooling compound extend horizontally or at right angles to the length of the mold, the letter T designating the inlet, U, the passages or cavities and V, the exhaust.

All parts of the mold excepting the refractory lining R, are composed of cast iron, steel or other metal or material. If desired a cover may be placed on the mold, the fastenings for same, as before mentioned, being designated by the letter S.

It is to be understood that the form of my invention herewith shown and described, is to be taken as a preferred example of the same, and that changes in the thickness of the walls, size of the passages, inlets or exhausts or of the material from which all parts or any part may be constructed may be resorted to without departing from the spirit of my invention or the scope of the subjoined claims.

In the use of my mold, the molten metal is poured from a ladle into such mold until same is filled to within about one inch from the top thereof. Within from two to five

minutes, which time, I have ascertained by experiment, the cooling compound is forced by pumping or otherwise through the inlet E into the passage F and up into the cavities H, in the zone A, resulting in the rapid cooling of that portion of the casting in the said zone A. This cooling of the said portion of the casting being greatest at the extreme bottom end thereof, because of the cooling compound being constantly renewed at this point, and gradually decreasing as the upper portion of the zone A is approached, by reason of the temperature of such cooling compound being constantly increased as it rises in the cavities H, it having been longer subjected to the heat of the casting. Said cooling compound then passes out through the exhausts J, constantly carrying with it the heat from the casting, which heat is dissipated in the surrounding atmosphere. As before stated, such cooling compound is unceasingly renewed, until the casting is wholly congealed.

As the metal of the casting at the extreme bottom portion thereof cools, the resulting natural contraction leaves cavities in the metal, which, if unfilled, become permanent, but the metal above being still in the fluid state flows downward and completely fills such cavities. As before described, by reason of the increased temperature of the cooling compound in the middle and upper parts of the cavities H, and by reason of the increasingly refractory condition of the walls of the mold in the zone B and the zone C, the metal of the casting gradually cools from the bottom upward, and as it cools, the cavities formed, as aforesaid, by the natural contraction of the cooling metal, are continually filled, by the force of gravity, by the still fluid metal from above. This process is constantly being repeated toward the top of the casting, until the same is wholly congealed.

By experiment, I have ascertained that the zone A will occupy about one half of the length of the mold, the zone B, about one third of the length, and the zone C, the remainder.

From the foregoing description, it is obvious that my invention will provide a mold, suitable for the present equipment of mills, and which, by reason of the constantly accelerated radiation from the top downward, will cause all pipes etc. to be filled, as soon as formed, from the still molten metal from above.

Having thus described my invention, I claim,

1. A mold, having the side-walls of its lower portion provided with passages and cavities, whereby such lower portion may be artificially cooled, the side-walls of its middle portion solid and normal with normal heat radiation, and the side-walls of its

upper portion provided with refractory lining for protective purposes and for the artificial retention of heat.

2. A mold, the side-walls of which, are, in its lower portion provided with passages and cavities whereby artificial cooling may be effected, in its middle portion, normal and solid, and in its upper portion lined with refractory substances to retain heat,

10  
whereby the metal cast in such mold will remain in a molten state longest at the top thereof, and by the force of gravity descend and fill all cavities formed by the more rapid cooling below.

**WILLIAM R. BOSSINGER.**

Witnesses:

**T. J. MILLS,**  
**STELLA ALLEN.**